

[54] **REMOVAL OF LEAD FROM COLUMBIUM MINERAL CONCENTRATE**

[75] Inventors: Dan M. Kentro, New York, N.Y.; James W. Cole, Boulder City, Nev.

[73] Assignee: **Molybdenum Corporation of America**, Louviers, Colo.[22] Filed: **May 18, 1972**[21] Appl. No.: **254,406**[52] **U.S. Cl.** ..... **75/84, 75/1**[51] **Int. Cl.** ..... **C22b 1/00**[58] **Field of Search** ..... **75/84, 2, 1**[56] **References Cited**

## UNITED STATES PATENTS

|           |        |         |       |         |
|-----------|--------|---------|-------|---------|
| 2,030,357 | 2/1936 | Doom    | ..... | 75/84 X |
| 2,150,555 | 3/1939 | Leemans | ..... | 75/84 X |
| 2,518,863 | 8/1950 | Gardner | ..... | 75/84   |

|           |         |                       |         |
|-----------|---------|-----------------------|---------|
| 2,905,549 | 9/1959  | Taylor et al. ....    | 75/84   |
| 2,909,426 | 10/1959 | Rathmann et al. ....  | 75/84 X |
| 3,132,024 | 5/1964  | Matricardi ....       | 75/84   |
| 3,141,766 | 7/1964  | Burkin et al. ....    | 75/84 X |
| 3,188,200 | 6/1965  | Brothers ....         | 75/84   |
| 3,453,101 | 7/1969  | Takahashi et al. .... | 75/2    |

*Primary Examiner*—Richard D. Lovering*Assistant Examiner*—R. E. Schafer*Attorney, Agent, or Firm*—Sheridan, Ross & Fields[57] **ABSTRACT**

A process for removing lead from columbium bearing material, such as minerals and concentrates, which comprises heating the material to at least about 650°C with up to 50% by weight of an inorganic metal chloride, or ammonium chloride, alkaline earth metal chlorides being preferred.

**14 Claims, No Drawings**

## REMOVAL OF LEAD FROM COLUMBIUM MINERAL CONCENTRATE

### BACKGROUND OF THE INVENTION

The metal columbium is in demand for use as an alloying agent in carbon and alloy steels and in non-ferrous metals, in advanced airframe systems, and for other specialized uses. A number of applications for the metal require a high purity product which is low in lead content. For example, the ASTM specifications for ferrocolumbium alloy limit its lead content to less than 0.01% by weight. (Percentage compositions referred to hereinafter are by weight.)

A major source for columbium is the mineral pyrochlore in which the metal is present largely as columbate along with other metals in combined form, such as, barium, calcium, iron, lead, rare earths, sodium, thorium, tin, titanium and others.

The average lead content of pyrochlore mineral concentrate is about 0.3 - 1% and the columbium content is about 60% based on  $\text{Cb}_2\text{O}_5$ . The major percentage of all of these metal impurities can be separated from columbium in pyrochlore and other columbium-containing minerals by conventional beneficiation procedures, with the exception of lead. For example, a commercial columbium concentrate from pyrochlore contains about 58-60% of columbium as  $\text{Cb}_2\text{O}_5$  and from 0.2-1% of lead.

A ferrocolumbium alloy produced from a concentrate containing this much lead has a lead content from about 0.05-0.2%, far above the ASTM tolerance of 0.01%. If a concentrate could be produced having a lead content of 0.05% or less, ferrocolumbium alloy could be produced from it with a lead content meeting the ASTM specifications. Prior to this invention a columbium concentrate could not be produced having a lead content less than about 0.2-1%.

Accordingly, it is an object of this invention to provide a process for removing lead from columbium bearing material.

It is another object of this invention to provide a process for separating lead from columbium when they are present together in mixtures.

### STATEMENT OF THE INVENTION

A process for the removal of lead from columbium bearing material which comprises mixing columbium concentrate with up to 50% of an inorganic metal chloride or ammonium chloride, heating the mixture above about 650°C for a period sufficient to eliminate substantially all of the lead as lead compounds or otherwise.

### DETAILED DESCRIPTION OF THE INVENTION

In the specification and claims reference to lead as being removed, separated, eliminated, etc. from columbium-containing material includes lead in the form of lead compounds.

In practicing the invention, finely divided concentrate obtained from the beneficiation of pyrochlore including froth flotation, is first thoroughly mixed by conventional procedures with up to 50% of ammonium chloride or an inorganic metal chloride in solid form. The mixture is then transferred to a standard furnace equipped to provide temperatures up to about 1000°C and above where it is heated at a temperature of at least

650°C for a period of up to 2 hours for removal of lead. The treated concentrate is leached with water or dilute hydrochloric acid as necessary to remove excess inorganic metal chloride after which ferrocolumbium alloy is produced from the treated concentrate by conventional processes.

The particle size of the concentrate is not critical, the only requirement being that it be sufficiently small to provide uniform mixing with the chloride. The process is applicable to minerals, ores, and other materials in which columbium is present with lead.

The concentrate used is normally a commercial grade concentrate produced by standard beneficiation techniques including a final froth flotation step.

The preferred inorganic metal chlorides are the alkaline earth metal chlorides, particularly, the chlorides of calcium and magnesium. Other chlorides found to be satisfactory are those of ammonium, the alkali metals, rare earth metals, and iron. Obviously, mixtures of

these chlorides are operative. While the explanation for the surprising effect of almost complete removal of lead is not known, it appears that the presence of chlorine in the form of an inorganic metal chloride plays a significant role in removal of the lead through volatilization of lead or lead compounds. Inorganic metal chlorides in general are operative. The chloride may be formed in situ by adding reactants which react to form the chloride. For example, lime and hydrochloric acid may be added in amounts to produce the required amount of calcium chloride.

The inorganic metal chloride may be used in amounts up to 50% by weight of the mixture. The amount used will depend on various factors including the lead content and physical condition of the concentrate, chloride used, as well as economic factors. Amounts up to 50% have been used with success. The preferred amount is between about 20-50%.

The lower limit of the temperature range within which the concentrate is heated is critical and is about 650°C. It must be high enough to volatilize the lead or lead compounds present under the reaction conditions. The upper limit is not critical and is dependent upon economic feasibility considerations as respects process time, heat utilization, purity of the product, and others.

A preferred range is between 700°-1000°C.

The time for heating the concentrate will vary depending on a number of factors such as the lead content of the concentrate, the chloride used, the physical condition of the concentrate, and the desired purity of the product. Times between about 15-120 minutes are preferred.

The test results reported in the following tables were obtained from tests made in accordance with the above-described procedure. They were selected as illustrative but not limiting of the invention. The concentrate used in the examples contained 61.35% columbium as  $\text{Cb}_2\text{O}_5$  and 0.33% lead. Fifty gram samples of concentrate were used. The percent lead removed was calculated by analysis of the sample before and after treatment. For each test the time of roast, temperature at which the roast was performed, weight percent of chloride additive based on weight of the concentrate sample, and weight percent of lead eliminated are given under appropriate headings.

The test results of Table 1 are for tests selected to illustrate the operativeness of the process with various inorganic metal chlorides under varying reaction conditions.

TABLE 1

| Test No. | Chloride                              | Wt. % Chloride | Temperature | Roast Time (Min.) | Wt. % Pb Eliminated |
|----------|---------------------------------------|----------------|-------------|-------------------|---------------------|
| 1        | —                                     | —              | 1000°C      | 30                | 0                   |
| 2        | CaCl <sub>2</sub>                     | 50             | 1000°C      | 90                | 100                 |
| 3        | CaCl <sub>2</sub>                     | 50             | 1000°C      | 90                | 100                 |
| 4        | MgCl <sub>2</sub> .6 H <sub>2</sub> O | 50             | 1000°C      | 60                | 60                  |
| 5        | MgCl <sub>2</sub> .6 H <sub>2</sub> O | 100            | 1000°C      | 120               | 95                  |
| 6        | BaCl <sub>2</sub>                     | 50             | 1000°C      | 30                | 45                  |
| 7        | NaCl                                  | 50             | 1000°C      | 90                | 50                  |
| 8        | KCl                                   | 50             | 1000°C      | 60                | 60                  |
| 9        | NH <sub>4</sub> Cl                    | 50             | 1000°C      | 120               | 80                  |
| 10       | FeCl <sub>3</sub>                     | 50             | 1000°C      | 60                | 50                  |
| 11       | Rare Earth Chloride Mixture           | 10             | 1000°C      | 90                | 60                  |

Table 1 test results demonstrate operativeness of the process with a wide range of inorganic metal chlorides under variable reaction conditions thus demonstrating the equivalency of the inorganic metal chlorides. From 45-100% lead was eliminated using alkaline earth metal chlorides and 50% and above lead elimination was obtained with the other metal chlorides.

The tests for which results are presented in Table 2 were selected to demonstrate the operativeness of the process when the chloride additive is formed in situ.

TABLE 2

| Test No. | Reactants | Amount of Reactants | Temperature | Roast Time (Min.) | Wt. % Pb Eliminated |
|----------|-----------|---------------------|-------------|-------------------|---------------------|
| 1        | HCl       | 25 cc               | 1000°C      | 90                | 85                  |
| 2        | CaO       | 10 gms.             |             |                   |                     |
|          | NaCl      | 30%                 | 1000°C      | 90                | 70                  |
|          | CaO       | 15%                 |             |                   |                     |

The results of Table 2 illustrate that the process operates with up to 85% elimination of lead when the chloride additive is formed in situ through the addition of reactants which react to form the chloride.

The results shown in Table 3 are for tests conducted to demonstrate the effect of varying the amounts of the chloride additive while maintaining the temperature and roast time constant.

TABLE 3

| Test No. | Chloride          | Wt. % Chloride | Temp.  | Roast Time (Min.) | Wt. % Pb Eliminated |
|----------|-------------------|----------------|--------|-------------------|---------------------|
| 1        | CaCl <sub>2</sub> | 5              | 1000°C | 90                | 45                  |
| 2        | do.               | 10             | do.    | do.               | 70                  |
| 3        | do.               | 20             | do.    | do.               | 75                  |
| 4        | do.               | 30             | do.    | do.               | 100                 |
| 5        | do.               | 40             | do.    | do.               | 100                 |
| 6        | do.               | 10             | 700°C  | do.               | 30                  |
| 7        | do.               | 20             | do.    | do.               | 50                  |
| 8        | do.               | 30             | do.    | do.               | 50                  |
| 9        | do.               | 40             | do.    | do.               | 50                  |

The results of Table 3 show that for a typical inorganic metal chloride, amounts from 5-40% can be used within the operable temperature and roast time ranges with 45-100% lead elimination.

The results of Table 4 below are for tests made to investigate the effect of varying the roast time while keeping the temperature and amount of chloride additive constant.

TABLE 4

| Test No. | Wt. % Chloride                                 | Temperature | Roast Time (Min.) | Wt. % Pb Eliminated |
|----------|------------------------------------------------|-------------|-------------------|---------------------|
| 1        | 30                                             | 1000°C      | 30                | 80                  |
| 2        | do.                                            | do.         | 45                | 95                  |
| 3        | do.                                            | do.         | 60                | 100                 |
| 4        | do.                                            | do.         | 75                | 100                 |
| 5        | do.                                            | do.         | 90                | 100                 |
| 6        | 5% NH <sub>4</sub> Cl<br>10% CaCl <sub>2</sub> | do.         | 120               | 70                  |

15 From the above test results it is apparent that use of roast times for a typical chloride additive within the preferred range of 30-120 minutes produces high percentage elimination of lead. Test No. 6 also illustrates the effectiveness of mixtures of the chlorides.

20 Test results are presented in Table 5 below from tests conducted to examine the effect of varying the process temperature while maintaining the amount of chloride additive and roast time constant.

TABLE 5

| Test No. | Chloride          | Wt. % Chloride | Temp. | Roast Time (Min.) | Wt. % Pb Eliminated |
|----------|-------------------|----------------|-------|-------------------|---------------------|
| 1        | CaCl <sub>2</sub> | 30             | 950°C | 90                | 100                 |
| 2        | do.               | do.            | 900°C | do.               | 88                  |
| 3        | do.               | do.            | 850°C | do.               | 94                  |
| 4        | do.               | do.            | 800°C | do.               | 77                  |
| 5        | do.               | do.            | 750°C | do.               | 63                  |
| 6        | do.               | do.            | 700°C | do.               | 50                  |

35 From the results of Table 5 it can be observed that for a typical chloride additive the operable temperature range is above about 700°C for 50% elimination of lead and above with 100% elimination obtained as the temperature approaches the preferred upper limit of 1,000°C.

40 The invention provides an economically feasible process for the elimination of lead from columbium concentrates. Concentrates are produced from which ferrocolumbium alloys can be made containing less than 0.01% lead, well within the ASTM specifications. The process can be economically used to separate lead from columbium in other applications in which such an effective separation may not be required, such as rough separation in unconcentrated ores and minerals, and other materials.

What is claimed is:

1. A process for removing lead from columbium mineral concentrates which comprises:
  - a. adding to the columbium mineral concentrates an inorganic chloride selected from the group consisting of alkaline earth metal chlorides, alkali metal chlorides, iron chlorides, rare earth metal chlorides, and ammonium chloride, and
  - b. heating the mixture of (a) at a temperature of at least 650°C for a period sufficient to remove substantially all of the lead from the columbium bearing mineral concentrates.
2. The process of claim 1 in which the amount of inorganic chloride added is up to about 50% by weight of the mixture.
3. The process of claim 2 in which the mixture is heated for a period of at least fifteen minutes.
4. The process of claim 1 in which the inorganic chloride is calcium chloride.
5. The process of claim 1 in which the inorganic chloride is magnesium chloride.
6. The process of claim 1 in which the inorganic chloride is ammonium chloride.
7. The process of claim 1 in which the inorganic chloride is barium chloride.
8. The process of claim 1 in which the inorganic chloride is potassium chloride.

9. The process of claim 1 in which the inorganic metal chloride is iron chloride.
10. The process of claim 1 in which the inorganic metal chloride is a rare earth metal chloride.
11. A process for removing lead from columbium mineral concentrates which comprises:
  - a. mixing with the columbium mineral concentrates in a finely divided state a finely divided solid inorganic chloride selected from the group consisting of alkaline earth metal chlorides, alkali metal chlorides, iron chlorides, rare earth metal chlorides, and ammonium chloride, and mixtures thereof, in an amount up to about 50 percent by weight of the mixture, and
  - b. heating the mixture at a temperature above about 650°C for a period of at least 15 minutes.
12. The process of claim 11 in which the mixture is heated from about 700°C-1000°C for a period from about 30-120 minutes.
13. The process of claim 12 in which excess inorganic metal salts are washed from the treated mixture.
14. The process of claim 11 in which the inorganic chloride is formed in situ by adding reactants which react under the reaction conditions to form the inorganic chloride.

\* \* \* \* \*

30

35

40

45

50

55

60

65